

# United States Patent

[11] 3,628,978

[72] Inventor **Edward C. Yackel**  
**Pittsford, N.Y.**  
[21] Appl. No. **761,852**  
[22] Filed **Sept. 23, 1968**  
[45] Patented **Dec. 21, 1971**  
[73] Assignee **Eastman Kodak Company**  
**Rochester, N.Y.**

3,186,842 6/1965 De Haes et al. .... 96/33 X  
3,278,958 10/1966 Regan et al. .... 96/33 X  
3,300,306 1/1967 Sevens et al. .... 96/33 X  
**FOREIGN PATENTS**  
934,693 8/1963 Great Britain ..... 96/29

*Primary Examiner*—Alfred L. Leavitt  
*Assistant Examiner*—Edward G. Whitby  
*Attorneys*—W. H. J. Kline, B. D. Wiese and H. E. Byers

[54] **METHOD OF NUCLEATING ALUMINUM**  
7 Claims, No Drawings

[52] U.S. Cl. .... 117/34,  
117/50, 117/130 R, 96/29, 96/33  
[51] Int. Cl. .... **B44d1/092**,  
B44d 1/02  
[50] Field of Search ..... 117/50, 34,  
130 R; 96/29, 33

**ABSTRACT:** Silver precipitating nuclei are deposited on a grained aluminum support such that said support can be used as a photolithographic receiving surface in a silver salt diffusion process by contacting the support with an alkaline bath and then contacting with an aqueous silver salt solution. In an alternative one-step treatment, an alkaline solution containing the silver salt is used.

[56] **References Cited**

UNITED STATES PATENTS

2,390,944 12/1945 King ..... 117/50 X

## METHOD OF NUCLEATING ALUMINUM

This invention relates to a method of preparing lithographic printing forms, particularly to lithographic printing plates made photographically.

The invention is concerned with the production of metallic plates for use in making lithographic printing plates by the silver salt diffusion process. As explained in British Pat. specification, Ser. No. 934,691, the silver salt diffusion process is a widely used commercial process wherein an imagewise exposed silver halide emulsion layer is developed in the presence of a silver halide solvent in such a manner that the undeveloped silver halide diffuses into the adjacent receiving sheet, where it is developed to give the desired image. The development nuclei such as silver nuclei deposited on the receiving sheet receive the developed silver from the diffusing silver halide and thus an image is formed thereon.

When using such a receiving sheet or support in lithography, both water and a greasy ink are applied and the support is sufficiently hydrophilic to accept water preferentially to the greasy ink, while the oleophilic image accepts ink preferentially to the water. Hence, to obtain good prints it is necessary that the difference in hydrophilic and oleophilic properties of the image and the background surface of the receiving sheet be sufficiently great that when water and ink are applied, the image will accept sufficient ink without the background accepting any ink at all.

The practice in making a photolithographic printing plate is to produce an oleophilic image on hydrophilic support which can be put into an inking machine whereby large numbers, up to 20,000 copies can usually be made very rapidly from the one plate.

In known processes wherein a silver image is formed on a receiving sheet by the silver salt diffusion process described above, it is usual to apply to the receiving surface on which the desired silver image is formed a gelatin solution containing both the development nuclei such as silver and a colloidal binder in which the nuclei are embedded. However, it is not possible to use the image developed therein as a lithographic printing plate because on wetting the layer for the purpose of making the nonsilver areas oleophobic, the gelatin of the silver areas is also rendered oleophobic. Thus, the silver image formed on the support does not accept sufficient ink to serve as a useful lithographic printing plate.

To remedy this very serious problem, extensive research has been and is presently underway to discover commercially practicable methods whereby development nuclei can be deposited on a satisfactory receiving surface without the use of a gelatin binder. As described in the aforementioned British Pat. specification, it has been found that a suitably grained and/or anodized aluminum sheet provides an excellent hydrophilic receiving surface for the development nuclei.

Various experimental tests have been conducted on such an aluminum support on which silver nuclei have been deposited. Although it has been established that aluminum receiving sheets containing silver nuclei deposited thereon are very satisfactory and are especially useful in the production of silver salt sensitized lithographic printing plates, it has also been recognized that the deposition of the nuclei on the receiving sheet (or nucleation of the receiving sheets as it is often referred to in the art) is a rather involved and somewhat uncertain process in which the interdependence of the various operations such as graining, anodizing, and application of the nuclei are not well understood and frequently result in an unsatisfactory material.

In other known processes such as that described in British Pat. specification, Ser. No. 934,692, nucleation of anodized and/or grained metallic surfaces requires treatment of the metallic surface with an aqueous colloidal dispersion of silver or gold particles. Although satisfactory results have been obtained by this process, the process is limited to aqueous colloidal dispersions of the element to be deposited on the receiving surface. Thus, use of the water-soluble silver salts such as silver nitrate and silver acetate, etc. which are the silver salts

generally utilized and preferred in commercial lithographic processes is prohibited.

According to one aspect of the present invention there is provided a method of depositing development nuclei on a grained aluminum support which comprises the steps of treating said grained aluminum support with an alkaline bath and subjecting said aluminum support to further treatment with an aqueous silver salt solution, thereby providing a nucleated aluminum support adaptable for use as a lithographic receiving sheet. In accordance with a preferred embodiment of the present invention the above recited steps of treating the grained aluminum support with an alkaline bath and then subjecting said grained aluminum support to further treatment with an aqueous silver salt solution can advantageously be performed simultaneously by initially dissolving the silver salt in the alkaline bath, thus yielding a single step process.

Several important aspects of the present invention should be particularly noted. First, it can be seen that the present invention requires only that the aluminum support be grained. Anodizing the support is unnecessary. Secondly, no colloidal binder is used. Treatment of the aluminum support with a colloidal dispersion of the element to be deposited thereon is eliminated; thus the commercially preferred water-soluble silver salts can be used. And fourth, the entire process, either the two step or the one step embodiment, can be accomplished in no more than 60 seconds. Thus, not only is the process of the present invention simple and reliable, but the extreme rapidity of the entire process represents a clear advance over known prior art techniques.

It has been found that the soluble silver salt contained dissolved in the aqueous bath used according to the present invention can be an inorganic, water-soluble salt such as silver nitrate, silver nitrite, silver sulfate, silver perchlorate, and the like, or it can be an organic silver salt such as silver acetate or silver lactate. Although the silver lactate, silver nitrate or silver acetate salts are preferred, it is believed that almost any water-soluble silver salt would give useful results. Other cations can also be used instead of silver or in addition to silver, provided they are more electropositive than aluminum.

The foregoing silver salts are especially useful in the above-described two step embodiment of the present invention wherein a grained aluminum support is first bathed in an alkaline solution followed by further bathing in the aqueous silver salt solution. In this embodiment the step of bathing in an alkaline medium is readily accomplished through the use of a large number of suitable basic solutions. Aqueous solutions of the alkali and alkaline-earth metal hydroxides, oxides and anhydrides are useful. The only real limitation is of course that the particular basic material selected must be water-soluble. It has been found that 0.1 normal solutions of potassium, ammonium and sodium hydroxide serve as preferred alkaline baths. The concentration of the alkaline solution will vary depending on the desired pH. However, neither the concentration of basic material nor the particular degree of alkalinity is considered to be a critical factor. For instance, as noted above, preferred alkaline baths include an aqueous solution of a strong base such as sodium hydroxide as well as a weak base such as ammonium hydroxide. Alkaline solutions having a pH within the range of about 10 to 14 are acceptable for use according to the instant invention, including both the two step embodiment and the one-step embodiment discussed immediately hereinafter.

With respect to the above-described one-step embodiment of the present invention wherein the step of bathing the grained aluminum support in an alkaline bath is performed simultaneously with the further step of subjecting the aluminum support to bathing in an aqueous bath of soluble silver salt, it has been found preferable to use a bath containing a silver salt dissolved in ammonium hydroxide to which an aqueous solution of sodium hydroxide has been subsequently added. Such a bath, wherein the silver salt, for example silver nitrate, is initially incorporated in the alkaline bath, upon contact with a grained aluminum support, results in a simple sin-

gle step process for the production of nucleated aluminum receiving sheets.

The method of the present invention for deposition of the development nuclei wherein the grained aluminum surface is treated by bathing in an aqueous solution of the silver salt ensures that the amount of the silver nuclei deposited on the surface per unit area is low. Silver salt solutions which may be used in either the above described one-step or two-step embodiments contain between about 0.2 and 0.0005 mole of silver salt per litre.

The grained aluminum support (or foil as it is referred to in the art) utilized in the present invention can be prepared by any of a variety of well-known techniques. A suitably grained sheet bearing a fine sharp lithographic grain has been produced by a chemical etching technique, a suitable material for conventional platemaking being that sold commercially by Addressograph Multigraph. Other suitable techniques include mechanical brushing or grinding. In any event, a wide variety of diverse techniques are known and can be utilized. The fact that the foil is grained ensures that the foil is sufficiently hydrophilic and also ensures the absence of contaminants such as oil.

The following examples are included for a further understanding of the invention:

#### EXAMPLE 1

A brushed-grained aluminum support 0.005 inch thick is placed in an 0.5 percent aqueous bath of sodium hydroxide for 30 seconds at room temperature and the excess removed by water rinse.

Immediately, thereafter, the brushed grained aluminum support is placed in a 0.1 N aqueous silver acetate bath for 30 seconds at room temperature, rinsed and dried.

The aforesaid nucleated aluminum support is then coated with an emulsion, contact exposed to a line positive, developed and further treated as described in British Pat. specification, Ser. No. 934,691, after which its press performance is that of a satisfactory lithographic printing plate.

#### EXAMPLE 2

In this example, a nucleated aluminum foil is prepared according to the process of example 1 except a solution of 0.1 N aqueous silver lactate is substituted for the aqueous silver acetate bath.

#### EXAMPLE 3

In this example, a nucleated aluminum foil is prepared according to the process of example 1 except a solution of 0.1 N aqueous silver nitrate is substituted for the aqueous silver acetate bath.

#### EXAMPLE 4

In this example, a nucleated aluminum foil is prepared according to the process of example 1 except a solution of 0.5 percent aqueous potassium hydroxide is substituted for the sodium hydroxide bath.

#### EXAMPLE 5

In this example, concentrated ammonium hydroxide is added to 0.1 N silver nitrate in sufficient excess quantity to

form silver hydroxide and dissolve it. To this solution is added a 0.1 N solution of sodium hydroxide equivalent to the silver. The resultant aqueous alkaline solution already containing the silver salt completely dissolved therein is then used as a bathing solution. That is, a grained aluminum foil identical to that described in example 1 is bathed in the alkaline solution for one minute at room temperature, rinsed and dried.

The resultant grained aluminum support having silver nuclei deposited thereon is then further treated as described in example 1 above, the result of which is the production of a satisfactory lithographic printing plate.

The invention has been described in detail with particular reference to preferred embodiments thereof, but it will be understood that variations and modifications can be effected within the spirit and scope of the invention as described hereinabove and as set forth in the appended claims.

I claim:

1. A method of depositing development nuclei on a grained aluminum support which comprises the steps of treating said 20 grained aluminum support with an aqueous bath selected from the class consisting of the alkali and alkaline earth metal hydroxides and oxides and ammonium hydroxide baths and subjecting said aluminum support to further treatment with an aqueous silver salt solution, thereby providing a nucleated aluminum support adaptable for use as a lithographic receiving sheet.
2. A method of depositing development nuclei on a grained aluminum support according to claim 1 wherein the steps of treating the grained aluminum support with an aqueous bath 30 selected from the class consisting of the alkali and alkaline earth metal hydroxides and oxides and ammonium hydroxide baths and then subjecting said grained aluminum support to treatment with an aqueous silver salt solution are performed simultaneously by initially dissolving the silver salt in said bath thereby yielding a single step process.
3. A method for depositing development nuclei on a grained aluminum support according to claim 2 wherein the said bath consists of an alkaline silver nitrate solution containing ammonium hydroxide and sodium hydroxide.
- 40 4. A method of depositing development nuclei on a grained aluminum support according to the method of claim 1 wherein said bath is a member selected from the group consisting of an aqueous solution of potassium hydroxide, an aqueous solution of ammonium hydroxide, and an aqueous solution of sodium hydroxide.
- 45 5. A method of depositing development nuclei on a grained aluminum support according to the method of claim 1 wherein the silver salt dissolved in said aqueous silver salt solution is a member selected from the group consisting of silver nitrate, silver acetate, and silver lactate.
- 50 6. A method of depositing development nuclei on a grained aluminum support according to the method of claim 1 wherein the said bath is a member selected from the group consisting of an aqueous solution of sodium hydroxide, an aqueous solution of potassium hydroxide, and an aqueous solution of ammonium hydroxide; and wherein the silver salt dissolved in said aqueous silver salt solution is a member selected from the group consisting of silver acetate, silver nitrate, and silver lactate.
- 55 60 7. A method of depositing development nuclei on a grained aluminum support according to the method of claim 6 wherein said silver salt is silver nitrate.

\* \* \* \* \*